



US007300726B1

(12) **United States Patent**  
**Patel et al.**

(10) **Patent No.:** **US 7,300,726 B1**  
(45) **Date of Patent:** **Nov. 27, 2007**

(54) **MULTI-LAYER IMAGEABLE ELEMENT  
WITH IMPROVED PROPERTIES**

(75) Inventors: **Jayanti Patel**, Fort Collins, CO (US);  
**Shashikant Saraiya**, Fort Collins, CO (US); **Ting Tao**, Fort Collins, CO (US)

(73) Assignee: **Eastman Kodak Company**, Rochester, NY (US)

(\*) Notice: Subject to any disclaimer, the term of this patent is extended or adjusted under 35 U.S.C. 154(b) by 0 days.

(21) Appl. No.: **11/551,259**

(22) Filed: **Oct. 20, 2006**

(51) **Int. Cl.**

**G03F 7/095** (2006.01)  
**G03F 7/11** (2006.01)  
**G03F 7/30** (2006.01)  
**G03F 7/039** (2006.01)

(52) U.S. Cl. .... **430/15**; 430/271.1; 430/302;  
430/306; 430/309; 430/326; 430/964

(58) **Field of Classification Search** .... **430/271.1**,  
430/964, 306, 309, 302, 326, 15  
See application file for complete search history.

(56) **References Cited**

U.S. PATENT DOCUMENTS

6,294,311 B1 9/2001 Shimazu et al.

|                 |         |                              |
|-----------------|---------|------------------------------|
| 6,352,811 B1    | 3/2002  | Patel et al.                 |
| 6,352,812 B1    | 3/2002  | Shimazu et al.               |
| 6,358,669 B1    | 3/2002  | Savariar-Hauck et al.        |
| 6,528,228 B2    | 3/2003  | Hauck et al.                 |
| 6,593,055 B2    | 7/2003  | Shimazu et al.               |
| 7,049,045 B2    | 5/2006  | Kitson et al.                |
| 7,060,415 B2 *  | 6/2006  | Kitson et al. .... 430/271.1 |
| 7,144,661 B1 *  | 12/2006 | Ray et al. .... 430/15       |
| 7,186,482 B2 *  | 3/2007  | Kitson et al. .... 430/15    |
| 2002/0160299 A1 | 10/2002 | Asawa et al.                 |
| 2004/0067432 A1 | 4/2004  | Kitson et al.                |

\* cited by examiner

*Primary Examiner*—Richard L. Schilling

(74) *Attorney, Agent, or Firm*—J. Lanny Tucker

(57) **ABSTRACT**

Positive-working imageable elements comprise a radiation absorbing compound and inner and outer layers on a substrate having a hydrophilic surface. The inner layer comprises a combination of two different polymeric binders one of which has an acid number of at least 30, which combination of polymers provides improved post-development bakeability (more quickly baked or cured at lower temperatures) and desired digital speed with no loss in chemical resistance.

**21 Claims, No Drawings**

## 1

MULTI-LAYER IMAGEABLE ELEMENT  
WITH IMPROVED PROPERTIES

## FIELD OF THE INVENTION

This invention relates to positive-working, multi-layer imageable elements that have various improved properties in imaging and post-development bakeability. It also relates to methods of using these elements to obtain lithographic printing plates and images therefrom.

## BACKGROUND OF THE INVENTION

In conventional or "wet" lithographic printing, ink receptive regions, known as image areas, are generated on a hydrophilic surface. When the surface is moistened with water and ink is applied, the hydrophilic regions retain the water and repel the ink, and the ink receptive regions accept the ink and repel the water. The ink is transferred to the surface of a material upon which the image is to be reproduced. For example, the ink can be first transferred to an intermediate blanket that in turn is used to transfer the ink to the surface of the material upon which the image is to be reproduced.

Imageable elements useful to prepare lithographic printing plates typically comprise an imageable layer applied over the hydrophilic surface of a substrate. The imageable layer includes one or more radiation-sensitive components that can be dispersed in a suitable binder. Alternatively, the radiation-sensitive component can also be the binder material. Following imaging, either the imaged regions or the non-imaged regions of the imageable layer are removed by a suitable developer, revealing the underlying hydrophilic surface of the substrate. If the imaged regions are removed, the element is considered as positive-working. Conversely, if the non-imaged regions are removed, the element is considered as negative-working. In each instance, the regions of the imageable layer (that is, the image areas) that remain are ink-receptive, and the regions of the hydrophilic surface revealed by the developing process accept water and aqueous solutions, typically a fountain solution, and repel ink.

Imaging of the imageable element with ultraviolet and/or visible radiation is typically carried out through a mask that has clear and opaque regions. Imaging takes place in the regions under the clear regions of the mask but does not occur in the regions under the opaque mask regions. If corrections are needed in the final image, a new mask must be made. This is a time-consuming process. In addition, dimensions of the mask may change slightly due to changes in temperature and humidity. Thus, the same mask, when used at different times or in different environments, may give different results and could cause registration problems.

Direct digital imaging has obviated the need for imaging through a mask and is becoming increasingly important in the printing industry. Imageable elements for the preparation of lithographic printing plates have been developed for use with infrared lasers. Thermally imageable, multi-layer elements are described, for example, in U.S. Pat. Nos. 6,294,311 (Shimazu et al.), 6,352,812 (Shimazu et al.), 6,593,055 (Shimazu et al.), 6,352,811 (Patel et al.), 6,358,669 (Savarier-Hauck et al.), and 6,528,228 (Savarier-Hauck et al.), and U.S. Patent Application Publication 2004/0067432 A1 (Kitson et al.).

## 2

U.S. Pat. No. 7,049,045 (Kitson et al.) describes multi-layer, positive-working imageable elements having improved resistant to press chemicals and that can be baked to increase press run length.

5

## PROBLEM TO BE SOLVED

Imaged multi-layer, positive-working elements are often baked after development to increase their on-press run length. While the known imageable elements demonstrate excellent imaging and printing properties, there is a need to improve the post-development bakeability of imaged elements while increasing imaging sensitivity (speed) and maintaining resistance to press chemicals. In particular, it is desired to reduce the baking temperature and time while maintaining on-press run length.

## SUMMARY OF THE INVENTION

20 This invention provides a positive-working imageable element comprising a radiation absorbing compound and a substrate having a hydrophilic surface, and having on the substrate, in order:

25 an inner layer composition comprising first and second polymeric binders, and

an ink receptive outer layer,

provided that upon thermal imaging, the exposed regions of the element are removable by an alkaline developer,

30 wherein the first polymeric binder has an acid number of at least 30 and comprises recurring units comprising acidic groups, and

35 the second polymeric binder comprises recurring units derived from an N-alkoxymethyl (alkyl)acrylamide, a hydroxymethyl (meth)acrylamide, an alkoxyethyl (alkyl) acrylate, or any combination thereof.

In another aspect, this invention provides a method for forming an image comprising:

40 A) thermally imagewise exposing the positive-working imageable element of this invention,

45 thereby forming an imaged element with exposed and non-exposed regions,

B) contacting the imaged element with an alkaline developer to remove only the exposed regions, and

C) optionally but preferably, baking the imaged and developed element in a manner as described below.

The multi-layer imageable elements of this invention have been found to have improved post-development bakeability (or curability) while they also have fast digital speed and desirable resistance to press chemicals. In particular, good on-press run length is possible even if the imaged and developed element is baked (or cured) as lower than normal temperatures and times.

55 DETAILED DESCRIPTION OF THE  
INVENTION

## Definitions

Unless the context indicates otherwise, when used herein, the terms "imageable element" and "printing plate precursor" are meant to be references to embodiments of the present invention.

In addition, unless the context indicates otherwise, the various components described herein such as the "first polymeric binder" and "second polymeric binder" used in the inner layer, "radiation absorbing compound", and similar terms also refer to mixtures of such components. Thus, the

use of the article "a", "an", or "the" is not necessarily meant to refer to only a single component.

Unless otherwise indicated, percentages refer to percentages by dry weight.

"Acid number" (or acid value) is measured as mg KOH/g using known methods.

For clarification of definitions for any terms relating to polymers, reference should be made to "Glossary of Basic Terms in Polymer Science" as published by the International Union of Pure and Applied Chemistry ("IUPAC"), *Pure Appl. Chem.* 68, 2287-2311 (1996). However, any definitions explicitly set forth herein should be regarded as controlling.

Unless otherwise indicated, the term "polymer" refers to high and low molecular weight polymers including oligomers and includes homopolymers and copolymers.

The term "copolymer" refers to polymers that are derived from two or more different monomers. That is, they comprise recurring units having at least two different chemical structures.

The term "backbone" refers to the chain of atoms in a polymer to which a plurality of pendant groups are attached. An example of such a backbone is an "all carbon" backbone obtained from the polymerization of one or more ethylenically unsaturated polymerizable monomers. However, other backbones can include heteroatoms wherein the polymer is formed by a condensation reaction or some other means.

#### Uses

The multi-layer imageable elements can be used in a number of ways. The preferred use is as precursors to lithographic printing plates as described in more detail below. However, this is not meant to be the only use of the present invention. For example, the imageable elements can also be used in photomask lithography and imprint lithography, and to make chemically amplified resists, printed circuit boards, and microelectronic and microoptical devices. The formulation used in the inner layer containing first and second polymeric binders may have other non-imaging uses such as in paint compositions.

#### Imageable Element

In general, the imageable element of this invention comprises a substrate, an inner layer (also known as an "under-layer"), and an outer layer (also known as a "top layer") disposed over the inner layer. Before thermal imaging, the outer layer is not removable by an alkaline developer, but after thermal imaging, the imaged (exposed) regions of the outer layer are removable by the alkaline developer. The inner layer is also removable by the alkaline developer. A radiation absorbing compound, generally an infrared radiation absorbing compound (defined below), is present in the imageable element. Preferably, this compound is in the inner layer exclusively, but optionally it can also be in a separate layer between the inner and outer layers.

The imageable elements are formed by suitable application of an inner layer composition onto a suitable substrate. This substrate can be an untreated or uncoated support but it is usually treated or coated in various ways as described below prior to application of the inner layer composition. The substrate generally has a hydrophilic surface or at least a surface that is more hydrophilic than the outer layer composition. The substrate comprises a support that can be composed of any material that is conventionally used to prepare imageable elements such as lithographic printing plates. It is usually in the form of a sheet, film, or foil, and is strong, stable, and flexible and resistant to dimensional change under conditions of use. Typically, the support can be

any self-supporting material including polymeric films (such as polyester, polyethylene, polycarbonate, cellulose ester polymer, and polystyrene films), glass, ceramics, metal sheets or foils, or stiff papers (including resin-coated and metallized papers), or a lamination of any of these materials (such as a lamination of an aluminum foil onto a polyester film). Metal supports include sheets or foils of aluminum, copper, zinc, titanium, and alloys thereof.

Polymeric film supports may be modified on one or both 10 surfaces with a "subbing" layer to enhance hydrophilicity, or paper supports may be similarly coated to enhance planarity. Examples of subbing layer materials include but are not limited to, alkoxy silanes, amino-propyl triethoxysilanes, glycidioxypropyl-triethoxysilanes, and epoxy functional polymers, as well as conventional hydrophilic subbing materials used in silver halide photographic films (such as gelatin and other naturally occurring and synthetic hydrophilic colloids and vinyl polymers including vinylidene chloride copolymers).

15 A preferred substrate is composed of an aluminum support that may be treated using techniques known in the art, including physical graining, electrochemical graining, chemical graining, and anodizing. Preferably, the aluminum sheet has been subjected to electrochemical graining and is anodized with sulfuric acid or phosphoric acid.

An interlayer may be formed by treatment of the aluminum support with, for example, a silicate, dextrine, calcium zirconium fluoride, hexafluorosilicic acid, an alkali phosphate solution containing an alkali halide (such as sodium fluoride), poly(vinyl phosphonic acid) (PVPA), vinyl phosphonic acid copolymer, poly(acrylic acid), or acrylic acid copolymer. Preferably, the grained and anodized aluminum support is treated with PVPA using known procedures to improve surface hydrophilicity.

20 The thickness of the substrate can be varied but should be sufficient to sustain the wear from printing and thin enough to wrap around a printing form. Preferred embodiments include a treated aluminum foil having a thickness of from about 100 to about 600  $\mu\text{m}$ .

25 The backside (non-imaging side) of the substrate may be coated with antistatic agents and/or slipping layers or a matte layer to improve handling and "feel" of the imageable element.

The substrate can also be a cylindrical surface having the 30 various layer compositions applied thereon, and thus be an integral part of the printing press. The use of such imaged cylinders is described for example in U.S. Pat. No. 5,713,287 (Gelbart).

#### Inner Layer

The inner layer is disposed between the outer layer and the substrate and, typically, disposed directly on the substrate described above. The inner layer comprises a composition that includes a mixture of at least two classes of 35 polymeric binders. Polymeric binders of a first class are identified herein as "first polymeric binders" and similarly, polymeric binders of a second class are identified herein as "second polymeric binders". Additional polymeric binders (described below) are optional and may be useful. The combination of first and second polymeric binders provides the improved bakeability of the resulting imageable elements of this invention. There may be multiple polymeric binders present from each class of polymeric binders.

The first polymeric binder has an acid number of at least 40 30, preferably of at least 50, and more preferably from about 60 to about 200. The desired acid number is provided by including various acidic recurring acidic groups along the

polymeric backbone, usually as pendant acidic groups such as pendant carboxy, sulfo, sulfonate, phospho, phosphate, and sulfate groups in recurring monomeric units. Such acidic groups can be present as free acids or as ammonium salts. Preferably, the acidic groups are carboxy or phospho groups that are present as free acidic groups or precursor groups such as anhydrides, carboxylates, or phosphates. The acidic groups can be provided by monomers that are polymerized and incorporated as recurring units into the polymer, or they can be formed in the polymer backbone after the polymer has been made, such as by converting pendant anhydride or ester groups to pendant free acid groups such as carboxy, sulfo, or phospho groups.

In preferred embodiments, the first polymeric binders comprise recurring units derived from one or more carboxyaryl (alkyl)acrylamides, one or more (alkyl)acrylate phosphates [including alkylene glycol (alkyl)acrylate phosphates], one or more (meth)acrylic acids, or combinations thereof.

The first polymeric binder may also comprise recurring units derived from other ethylenically unsaturated polymerizable monomers including one or more ethylenically unsaturated polymerizable monomers that include pendant cyano groups, including but not limited to, (meth)acrylonitriles.

The term "carboxyaryl (alkyl)acrylamides" includes acrylamides as well as alkylacrylamides having alkyl groups replacing one or more of the hydrogen atoms on the vinyl group. The term "alkyl" group can have 1 to 6 carbon atoms and include but not be limited to, methyl, ethyl, iso-propyl, and benzyl groups, but preferably, the alkyl group is methyl or ethyl, and more preferably, it is methyl. The "aryl" group in such monomers is an aromatic carbocyclic group such as a phenyl or naphthyl group that can be substituted with one or more carboxy groups as well as one or more other substituents such as alkyl, alkenyl, and halo groups. Preferably, it is a phenyl group substituted with a single carboxy group (more preferably, in the 4-position). Preferred monomers of this type can be represented by the following Structure (A<sub>1</sub>):



wherein R<sub>1</sub> is the defined alkyl group, Ar is the defined aryl group, and n is 1 to 5. Most preferably, R<sub>1</sub> is hydrogen or methyl, Ar is phenyl, n is 1, and the carboxy group is in the 4-position on the phenyl group: that is, 4-carboxyphenyl (meth)acrylamide.

One or more (alkyl)acrylate phosphates include "acrylates" and "alkylacrylates" and can also be used to prepare the first polymeric binder. A preferred class of such monomers includes alkylene glycol (alkyl)acrylates. By the term "alkylene" we mean substituted or unsubstituted linear or branched hydrocarbon groups having 1 to 100 carbon atoms that are attached to an oxy group to form an "alkylene glycol" moiety. The "alkyl" group can be substituted or unsubstituted and have 1 to 6 carbon atoms. This class of monomers can also be represented by the following Structure (A<sub>2</sub>):



wherein R<sub>1</sub> is as defined above, Y is a carbon-oxygen bond or an —O-alkylene group wherein alkylene is as defined above, and M is a suitable monovalent cation such as hydrogen, ammonium ion, or an alkali metal ion. Preferably, M is hydrogen. More particularly, the alkylene group can be defined as —[O(CH<sub>2</sub>)<sub>m</sub>]<sub>p</sub> wherein m is 2 to 4 (preferably 2)

and p is 1 to 20 (preferably 1 to 5). Preferred monomers of this class include ethylene glycol or propylene glycol (meth)acrylate phosphates.

The term "(meth)acrylic acid" includes both methacrylic acid and acrylic acid as well as precursors thereof such as anhydrides.

Particularly useful first polymeric binders comprise recurring units derived from a (meth)acrylic acid, and one or more of carboxyphenyl (meth)acrylamide, an ethylene glycol or propylene glycol (meth)acrylate phosphate, or a combination thereof.

The first polymeric binder(s) can be further represented by the following Structure (I):



wherein A represents recurring units derived from a (meth) acrylic acid, carboxyaryl (alkyl)acrylamide, a (alkyl)acrylate phosphate, or a combination thereof, as defined above, B represents recurring units derived from one or more

20 different ethylenically unsaturated polymerizable monomers other than those used to obtain the A recurring units and optionally recurring units derived from (meth)acrylonitrile, x is from about 1 to about 70 mol % (preferably from about 5 to about 50 mol %), and y is from about 30 to about 99 mol % (preferably from about 50 to about 95 mol %), based on total recurring units.

Useful monomers from which the B recurring units can be derived include, but are not limited to, one or more (meth) acrylonitriles, (meth)acrylic acid esters, (meth)acrylamides, vinyl carbazole, styrene and styrenic derivatives thereof, N-substituted maleimides, maleic anhydride, vinyl acetate, vinyl ketones, vinyl pyridine, N-vinyl pyrrolidones, 1-vinylimidazole, vinyl polyalkylsilanes and combinations thereof.

The second polymeric binder comprises recurring units derived from an N-alkoxymethyl (alkyl)acrylamide, alkoxyethyl (alkyl)acrylate, hydroxymethyl (alkyl)acrylamide, or any combination thereof.

The term "alkoxy" refers to substituted or unsubstituted 40 alkoxy groups having 1 to 12 carbon atoms, and preferably from 1 to 6 carbon atoms. "Alkyl" is defined as described above for the first polymeric binder.

The second polymeric binder can also be represented by the following Structure (C<sub>1</sub>):



wherein R<sub>1</sub> is as defined above, X is —O— or —NH—, and R<sub>2</sub> is hydrogen or a substituted or unsubstituted alkyl group having 1 to 12 carbon atoms or substituted or unsubstituted aryl group having 6 or 10 carbon atoms in the ring, provided that when X is —O—, R<sub>2</sub> is not hydrogen. Preferably, R<sub>1</sub> is hydrogen or methyl, and R<sub>2</sub> is hydrogen or methyl. For example, monomers of this class include a methoxymethyl (meth)acrylamide, hydroxymethyl (meth)acrylamide, methoxymethyl (meth)acrylate, or any combination thereof.

The second polymeric binder can also be represented by the following Structure (II):



wherein C represents recurring units derived from an N-alkoxymethyl (alkyl)acrylamide, alkoxyethyl (alkyl)acrylate, hydroxymethyl (alkyl)acrylamide, or any combination thereof, D represents recurring units derived from one or more different ethylenically unsaturated polymerizable monomers other than those used to obtain the C recurring units, w is from about 5 to about 80 mol % (preferably from

about 10 to about 60 mol %), and z is from about 20 to about 95 mol % (preferably 40 to about 90 mol %), based on total recurring units.

Monomers from which the D recurring units can be derived include but are not limited to, one or more (meth) acrylic acid esters, (meth)acrylonitriles, (meth)acrylamides, vinyl carbazole, styrene and styrenic derivatives thereof, N-substituted maleimides, maleic anhydride, vinyl acetate, vinyl ketones, vinyl pyridine, N-vinyl pyrrolidones, 1-vinylimidazole, vinyl monomers having carboxy groups such as (meth)acrylic acid, vinyl polyalkylsilanes, and combinations thereof.

D preferably represents recurring units derived from one or more of an N-substituted maleimide, N-substituted (meth) acrylamide, unsubstituted (meth)acrylamide, methyl (meth) acrylate, benzyl (meth)acrylate, (meth)acrylonitrile, a styrenic monomer, and combinations thereof, and D can also represent recurring units derived from (meth)acrylic acid.

Particularly useful embodiments of this invention include imageable elements in which the first polymeric binder comprises recurring units derived from a (meth)acrylic acid, and one or more of 4-carboxyphenyl (meth)acrylamide, an ethylene glycol (meth)acrylate phosphate, or a combination thereof, and the second polymeric binder comprises recurring units derived from an N-alkoxymethyl (meth)acrylamide.

Most particularly useful first and second polymeric binders are described in the Examples below.

The first and second polymeric binders can be prepared using known starting materials (monomers and polymerization initiators) and solvents and reaction conditions. Representative synthetic methods are provided below before the Examples.

The total amount of first and second polymeric binders generally present in the inner layer composition is a coverage of from about 50 to about 99 weight %, and preferably at from about 70 to about 95 weight %, based on total dry inner layer weight. The amount of the first polymeric binder is generally from about 20 to about 90 weight % and preferably from about 20 to about 80 weight %. The amount of the second polymeric binder is generally from about 5 to about 80 weight % and preferably from about 10 to about 80 weight %. The weight ratio of the first polymeric binder to the second polymeric binder in the inner layer is generally from about 0.2:1 to about 20:1 and preferably from about 1:1 to about 10:1.

The inner layer composition can also be defined as "curable" upon heating at from about 160 to about 220° C. for from about 2 to about 5 minutes, or by overall infrared radiation exposure at from about 800 to about 850 nm. By "curable", we mean that the inner layer composition comprising the mixture of first and second polymeric binders is curable upon heating it at from about 160 to about 220° C. for from about 2 to about 5 minutes, or from overall infrared radiation exposure at from about 800 to about 850 nm. Such a cured inner layer composition then is not damaged or removed when contacted with PS Plate Image Remover, PE-3S (Kodak Polychrome Graphics-Japan and distributed by Dainippon Ink & Chemicals, Inv.) at ambient temperatures for up to 10 minutes.

Preferably, the inner layer composition further exclusively comprises a radiation absorbing compound (preferably an infrared radiation absorbing compound) that absorbs radiation at from about 600 to about 1400 nm and preferably at from about 700 to about 1200 nm, with minimal absorption at from about 300 to about 600 nm. This compound (sometimes known as a "photothermal conversion material"

or "thermal convertor") absorbs radiation and converts it to heat. This compound may be either a dye or pigment. Examples of useful pigments are ProJet 900, ProJet 860 and ProJet 830 (all available from the Zeneca Corporation).

Although a radiation absorbing compound is not necessary for imaging with a hot body, the imageable elements containing a radiation absorbing compounds may also be imaged with a hot body, such as a thermal head or an array of thermal heads.

Useful IR absorbing compounds also include carbon blacks including carbon blacks that are surface-functionalized with solubilizing groups are well known in the art. Carbon blacks that are grafted to hydrophilic, nonionic polymers, such as FX-GE-003 (manufactured by Nippon Shokubai), or which are surface-functionalized with anionic groups, such as CAB-O-JET® 200 or CAB-O-JET® 300 (manufactured by the Cabot Corporation) are also useful.

IR dyes (especially those that are soluble in an alkaline developer) are preferred to prevent sludging of the developer by insoluble material. Examples of suitable IR dyes include but are not limited to, azo dyes, squarylium dyes, croconate dyes, triarylamine dyes, thioazolium dyes, indolium dyes, oxonol dyes, oxazolium dyes, cyanine dyes, merocyanine dyes, phthalocyanine dyes, indocyanine dyes, indoaniline dyes, merostyryl dyes, indotricarbocyanine dyes, oxatricarbocyanine dyes, thiocyanine dyes, thiaticarbocyanine dyes, merocyanine dyes, cryptocyanine dyes, naphthalocyanine dyes, polyaniline dyes, polypyrrole dyes, polythiophene dyes, chalcogenopyrroloarylidene and bi(chalcogenopyrrolo) polymethine dyes, oxyindolizine dyes, pyrilium dyes, pyrazoline azo dyes, oxazine dyes, naphthoquinone dyes, anthraquinone dyes, quinoneimine dyes, methine dyes, arylmethine dyes, squaraine dyes, oxazole dyes, croconine dyes, porphyrin dyes, and any substituted or ionic form of the preceding dye classes. Suitable dyes are also described in numerous publications including U.S. Pat. Nos. 6,294,311 (noted above) and 5,208,135 (Patel et al.) and the references cited thereon, that are incorporated herein by reference.

Examples of useful IR absorbing compounds include ADS-830A and ADS-1064 (American Dye Source, Baie D'Urfe, Quebec, Canada), EC2117 (FEW, Wolfen, Germany), Cyasorb® IR 99 and Cyasorb® IR 165 (GPTGlendale Inc. Lakeland, Fla.), and IR Absorbing Dye A used in the Examples below.

Near infrared absorbing cyanine dyes are also useful and are described for example in U.S. Pat. Nos. 6,309,792 (Hauck et al.), 6,264,920 (Achilefu et al.), 6,153,356 (Urano et al.), 6,787,281 (Tao et al.), and 5,496,903 (Watanate et al.). Suitable dyes may be formed using conventional methods and starting materials or obtained from various commercial sources including American Dye Source (Canada) and FEW Chemicals (Germany). Other useful dyes for near infrared diode laser beams are described, for example, in U.S. Pat. No. 4,973,572 (DeBoer).

In addition to low molecular weight IR-absorbing dyes, IR dye moieties bonded to polymers can be used as well. Moreover, IR dye cations can be used, that is, the cation is the IR absorbing portion of the dye salt that ionically interacts with a polymer comprising carboxy, sulfo, phosphor, or phosphono groups in the side chains.

The radiation absorbing compound can be present in an amount of generally from about 5% to about 40% and preferably from about 7 to about 20%, based on the total inner layer dry weight. The particular amount needed for a given IR absorbing compound can be readily determined by one skilled in the art.

The inner layer can include other components such as surfactants, dispersing aids, humectants, biocides, viscosity builders, drying agents, defoamers, preservatives, antioxidants, colorants, and other polymers such as novolaks, resoles, or resins that have activated methylol and/or activated alkylated methylol groups as described for example in U.S. Pat. No. 7,049,045 (noted above).

The inner layer generally has a dry coating coverage of from about 0.5 to about 3.5 g/m<sup>2</sup> and preferably from about 1 to about 2.5 g/m<sup>2</sup>.

#### Outer Layer

The outer layer is disposed over the inner layer and in preferred embodiments there are no intermediate layers between the inner and outer layers. The outer layer becomes soluble or dispersible in the developer upon thermal exposure. It typically comprises one or more ink-receptive polymeric materials, known as polymer binders, and a dissolution inhibitor or colorant. Alternatively, or additionally, a polymer binder comprises polar groups and acts as both the binder and dissolution inhibitor.

Any polymer binders may be employed in the imageable elements if they have been previously used in outer layers of prior art multi-layer thermally imageable elements. For example, the polymer binders can be one or more of those described in U.S. Pat. Nos. 6,358,669 (Savariar-Hauck), 6,555,291 (Hauck), 6,352,812 (Shimazu et al.), 6,352,811 (Patel et al.), 6,294,311 (Shimazu et al.), 6,893,783 (Kitson et al.), and 6,645,689 (Jarek), U.S. Patent Application Publications 2003/0108817 (Patel et al) and 2003/0162126 (Kitson et al.), and WO 2005/018934 (Kitson et al.).

Preferably, the polymer binder in the outer layer is a light-insensitive, water-insoluble, aqueous alkaline developer-soluble, film-forming phenolic resin that has a multiplicity of phenolic hydroxyl groups. Phenolic resins have a multiplicity of phenolic hydroxyl groups, either on the polymer backbone or on pendent groups. Novolak resins, resol resins, acrylic resins that contain pendent phenol groups, and polyvinyl phenol resins are preferred phenolic resins. Novolak resins are more preferred.

Novolak resins are commercially available and are well known to those in the art. Novolak resins are typically prepared by the condensation reaction of a phenol, such as phenol, m-cresol, o-cresol, p-cresol, etc, with an aldehyde, such as formaldehyde, paraformaldehyde, acetaldehyde, etc. or ketone, such as acetone, in the presence of an acid catalyst. The weight average molecular weight is typically about 1,000 to 15,000. Typical novolak resins include, for example, phenol-formaldehyde resins, cresol-formaldehyde resins, phenol-cresol-formaldehyde resins, p-t-butylphenol-formaldehyde resins, and pyrogallol-acetone resins. Particularly useful novolak resins are prepared by reacting m-cresol, mixtures of m-cresol and p-cresol, or phenol with formaldehyde using conditions well known to those skilled in the art.

A solvent soluble novolak resin is one that is sufficiently soluble in a coating solvent to produce a coating solution that can be coated to produce an outer layer. In some cases, it may be desirable to use a novolak resin with the highest weight-average molecular weight that maintains its solubility in common coating solvents, such as acetone, tetrahydrofuran, and 1-methoxypropan-2-ol. Outer layers comprising novolak resins, including for example m-cresol only novolak resins (i.e. those that contain at least about 97 mol-% m-cresol) and m-cresol/p-cresol novolak resins that have up to 10 mol-% of p-cresol, having a weight average molecular weight of at least 10,000 and preferably at least

25,000, are preferred. Outer layers comprising m-cresol/p-cresol novolak resins with at least 10 mol-% of p-cresol, having a weight average molecular weight of about 8,000 up to about 25,000, may also be used. In some instances, novolak resins prepared by solvent condensation may be desirable. Outer layers comprising these resins are disclosed for example in U.S. Pat. No. 6,858,359 (Kitson, et al.).

Other useful phenolic resins are poly(vinyl phenol) resins that include polymers of one or more hydroxyphenyl containing monomers such as hydroxystyrenes and hydroxyphenyl (meth)acrylates. Other monomers not containing hydroxy groups can be copolymerized with the hydroxy-containing monomers. These resins can be prepared by polymerizing one or more of the monomers in the presence of a radical initiator or a cationic polymerization initiator using known reaction conditions. The weight average molecular weight ( $M_w$ ) of these polymers is from about 1000 to about 200,000 g/mol, and more preferably from about 1,500 to about 50,000 g/mol.

Examples of useful hydroxy-containing polymers include ALNOVOL SPN452, SPN400, HPN100 (Clariant GmbH), DURITE PD443, SD423A, SD126A (Borden Chemical, Inc.), BAKELITE 6866LB02, AG, 6866LB03 (Bakelite AG), KR 400/8 (Koyo Chemicals Inc.), HRJ 1085 and 2606 (Schenectady International, Inc.), and Lyncur CMM (Siber Hegner), all of which are described in U.S. Patent Application Publication 2005/0037280 (noted above). A particularly useful polymer is PD-140A described for the Examples below.

The outer layer can also include non-phenolic polymeric materials as film-forming binder materials in addition to or instead of the phenolic resins described above. Such non-phenolic polymeric materials include polymers formed from maleic anhydride and one or more styrenic monomers (that is styrene and styrene derivatives having various substituents on the benzene ring), polymers formed from methyl methacrylate and one or more carboxy-containing monomers, and mixtures thereof. These polymers can comprise recurring units derived from the noted monomers as well as recurring units derived from additional, but optional monomers [such as (meth)acrylates, (meth)acrylonitrile and (meth)acrylamides].

The polymers derived from maleic anhydride generally comprise from about 1 to about 50 mol % of recurring units derived from maleic anhydride and the remainder of the recurring units derived from the styrenic monomers and optionally additional polymerizable monomers.

The polymer formed from methyl methacrylate and carboxy-containing monomers generally comprise from about 80 to about 98 mol % of recurring units derived from methyl methacrylate. The carboxy-containing recurring units can be derived, for example, from acrylic acid, methacrylic acid, itaconic acid, maleic acid, and similar monomers known in the art.

The outer layer can also comprise one or more polymer binders having pendant epoxy groups sufficient to provide an epoxy equivalent weight of from about 130 to about 1000 (preferably from about 140 to about 750). "Epoxy equivalent weight" refers to the weight of the polymer (grams) divided by the number of equivalence of epoxy groups (number of moles) in the polymer. Any film-forming polymer containing the requisite pendant epoxy groups can be used including condensation polymers, acrylic resins, and urethane resins. The pendant epoxy groups can be part of the polymerizable monomers or reactive components used to make the polymers, or they can be added after polymerization using known procedures. Preferably, the outer layer

## 11

comprises one or more acrylic resins that are derived from one or more ethylenically unsaturated polymerizable monomers, at least one of which monomers comprises pendant epoxy groups.

Particularly useful polymers of this type have pendant epoxy groups attached to the polymer backbone through a carboxylic acid ester group such as a substituted or unsubstituted —C(O)O-alkylene, —C(O)O-alkylene-phenylene-, or —C(O)O-phenylene group wherein alkylene has 1 to 4 carbon atoms. Preferred ethylenically unsaturated polymerizable monomers having pendant epoxy groups useful to make these polymer binders include glycidyl acrylate, glycidyl methacrylate, 3,4-epoxycyclohexyl methacrylate, and 3,4-epoxycyclohexyl acrylate.

The epoxy-containing polymers can also comprise recurring units derived from one or more ethylenically unsaturated polymerizable monomers that do not have pendant epoxy groups including but not limited to, (meth)acrylates, (meth)acrylamides, vinyl ether, vinyl esters, vinyl ketones, olefins, unsaturated imides (such as maleimide), N-vinyl pyrrolidones, N-vinyl carbazole, vinyl pyridines, (meth)acrylonitriles, and styrenic monomers. Of these, the (meth)acrylates, (meth)acrylamides, and styrenic monomers are preferred and the styrenic monomers are most preferred. For example, a styrenic monomer could be used in combination with methacrylamide, acrylonitrile, maleimide, vinyl acetate, or N-vinyl pyrrolidone.

Still other useful polymeric binders for the outer layer include those having a polymer backbone and pendant sulfonamide groups such as pendant —X—C(=T)—NR—S(=O)<sub>2</sub>— groups that are attached to the polymer backbone, wherein X is oxy or amido, T is oxygen or sulfur, and R is hydrogen, halo, or an alkyl group having 1 to 6 carbon atoms.

The polymeric binders in the outer layer can also be branched hydroxystyrene polymers that include recurring units derived from 4-hydroxystyrene, which recurring units are further substituted with repeating 4-hydroxystyrene units positioned ortho to the hydroxy groups.

The one or more polymer binders are present in the outer layer in an amount of at least 60 weight %, and preferably from about 65 to about 99.5 weight %.

The outer layer generally and optionally comprises a dissolution inhibitor that functions as a solubility-suppressing component for the binder. Dissolution inhibitors generally have polar functional groups that are thought to act as acceptor sites for hydrogen bonding, such as with hydroxyl groups of the binder. Dissolution inhibitors that are soluble in the developer are most suitable. Alternatively, or additionally, the polymer binder may contain solubility-suppressing polar groups that function as the dissolution inhibitor. Useful dissolution inhibitor compounds are described for example in U.S. Pat. Nos. 5,705,308 (West, et al.), 6,060,222 (West, et al.), and 6,130,026 (Bennett, et al.).

Compounds that contain a positively charged (that is, quaternized) nitrogen atom useful as dissolution inhibitors include, for example, tetraalkyl ammonium compounds, quinolinium compounds, benzothiazolium compounds, pyridinium compounds, and imidazolium compounds. Representative tetraalkyl ammonium dissolution inhibitor compounds include tetrapropyl ammonium bromide, tetraethyl ammonium bromide, tetrapropyl ammonium chloride, and trimethylalkyl ammonium chlorides and trimethylalkyl ammonium bromides, such as trimethyloctyl ammonium bromide and trimethyldecyt ammonium chloride. Representative quinolinium dissolution inhibitor compounds include 1-ethyl-2-methyl quinolinium iodide, 1-ethyl-4-methyl

## 12

quinolinium iodide and cyanine dyes that comprise a quinolinium moiety such as Quinoline Blue. Representative benzothiazolium compounds include 3-ethyl-2(3H)-benzothiazolylidene)-2-methyl-1-(propenyl)benzothiazolium cationic dyes and 3-ethyl-2-methyl benzothiazolium iodide.

Diazonium salts are useful as dissolution inhibitor compounds and include, for example, substituted and unsubstituted diphenylamine diazonium salts, such as methoxy-substituted diphenylamine diazonium hexafluoroborates.

10 Representative sulfonic acid esters useful as dissolution inhibitor compounds include ethyl benzene sulfonate, n-hexyl benzene sulfonate, ethyl p-toluene sulfonate, t-butyl p-toluene sulfonate, and phenyl p-toluene sulfonate. Representative phosphate esters include trimethyl phosphate, triethyl phosphate, and tricresyl phosphate. Useful sulfones include those with aromatic groups, such as diphenyl sulfone. Useful amines include those with aromatic groups, such as diphenylamine and triphenylamine.

15 Keto-containing compounds useful as dissolution inhibitor compounds include, for example, aldehydes, ketones, especially aromatic ketones, and carboxylic acid esters. Representative aromatic ketones include xanthone, flavanones, flavones, 2,3-diphenyl-1-indenone, 1'-(2'-acet-25 onaphthonyl)benzoate, 2,6-diphenyl-4H-pyran-4-one and 2,6-diphenyl-4H-thiopyran-4-one. Representative carboxylic acid esters include ethyl benzoate, n-heptyl benzoate, and phenyl benzoate.

20 Other readily available dissolution inhibitors are triaryl-methane dyes, such as ethyl violet, crystal violet, malachite green, brilliant green, Victoria blue B, Victoria blue R, Victoria blue BO, BASONYL Violet 610. These compounds can also act as contrast dyes that distinguish the non-exposed regions from the exposed regions in the developed imageable element.

25 When a dissolution inhibitor compound is present in the outer layer, it typically comprises at least about 0.1 weight %, more generally from about 0.5 to about 30 weight %, and preferably from about 1 to about 15 weight %, based on the dry weight of the outer layer.

30 Alternatively, or additionally, the polymer binder in the outer layer can comprise polar groups that act as acceptor sites for hydrogen bonding with the hydroxy groups present in the polymeric material and, thus, act as both the binder and dissolution inhibitor. These derivatized polymeric materials can be used alone in the outer layer, or they can be combined with other polymeric materials and/or solubility-suppressing components. The level of derivatization should be high enough that the polymeric material acts as a dissolution inhibitor, but not so high that, following thermal imaging, the polymeric material is not soluble in the developer. Although the degree of derivatization required will depend on the nature of the polymeric material and the nature of the moiety containing the polar groups introduced into the polymeric material, typically from about 0.5 mol % to about 5 mol %, and preferably from about 1 mol % to about 3 mol %, of the hydroxyl groups will be derivatized.

35 One group of polymeric materials that comprise polar groups and function as dissolution inhibitors are derivatized phenolic polymeric materials in which a portion of the phenolic hydroxyl groups have been converted to sulfonic acid esters, preferably phenyl sulfonates or p-toluene sulfonates. Derivatization can be carried out by reaction of the 40 polymeric material with, for example, a sulfonyl chloride such as p-toluene sulfonyl chloride in the presence of a base such as a tertiary amine. A useful material is a novolak resin

## 13

in which from about 1 to about 3 mol % of the hydroxyl groups has been converted to phenyl sulfonate or p-toluene sulfonate (tosyl) groups.

Another group of polymeric materials that comprise polar groups and function as dissolution inhibitors are derivatized phenolic resins that contain the diazonaphthoquinone moiety. Polymeric diazonaphthoquinone compounds include derivatized resins formed by the reaction of a reactive derivative that contains diazonaphthoquinone moiety and a polymeric material that contains a suitable reactive group, such as a hydroxyl or amino group. Derivatization of phenolic resins with compounds that contain the diazonaphthoquinone moiety is known in the art and is described, for example, in U.S. Pat. Nos. 5,705,308 and 5,705,322 (both West, et al.). An example of a resin derivatized with a compound that comprises a diazonaphthoquinone moiety is P-3000 (available from PCAS, France) that is a naphthoquinone diazide of a pyrogallol/acetone resin.

To reduce ablation during imaging with infrared radiation, the outer layer is substantially free of radiation absorbing compounds, meaning that none of those compounds are purposely incorporated therein and insubstantial amounts diffuse into it from other layers. Thus, any radiation absorbing compounds in the outer layer absorb less than about 10% of the imaging radiation, preferably less than about 3% of the imaging radiation, and the amount of imaging radiation absorbed by the outer layer, if any, is not enough to cause ablation of the outer layer.

The outer layer can also include other components such as surfactants, dispersing aids, humectants, biocides, viscosity builders, drying agents, antifoaming agents, preservatives, antioxidants, colorants, and contrast dyes. Coating surfactants are particularly useful.

The outer layer generally has a dry coating coverage of from about 0.2 to about 2 g/m<sup>2</sup> and preferably from about 0.4 to about 1 g/m<sup>2</sup>.

Although not preferred, there may be a separate layer that is disposed between the inner and outer layers. This separate layer (or interlayer) can act as a barrier to minimize migration of radiation absorbing compounds from the inner layer to the outer layer. This interlayer generally comprises a polymeric material that is soluble in an alkaline developer. A preferred polymeric material of this type is a poly(vinyl alcohol). Generally, the interlayer should be less than one-fifth as thick as the inner layer and preferably less than one-tenth as thick as the outer layer.

#### Preparation of the Imageable Element

The imageable element can be prepared by sequentially applying an inner layer formulation over the surface of the substrate (and any other hydrophilic layers provided thereon), and then applying an outer layer formulation over the inner layer using conventional coating or lamination methods. It is important to avoid intermixing the inner and outer layer formulations.

The inner and outer layer formulations can be applied by dispersing or dissolving the desired ingredients in suitable coating solvents, and the resulting formulations are sequentially or simultaneously applied to the substrate using any suitable equipment and procedures, such as spin coating, knife coating, gravure coating, die coating, slot coating, bar coating, wire rod coating, roller coating, or extrusion hopper coating. The formulations can also be applied by spraying onto a suitable support (such as an on-press printing cylinder).

The selection of solvents used to coat both the inner and outer layers depends upon the nature of the polymeric

## 14

materials and other components in the formulations. To prevent the inner and outer layer formulations from mixing or the inner layer dissolving when the outer layer formulation is applied, the outer layer should be coated from a solvent in which the polymeric material(s) of the inner layer are insoluble. Generally, the inner layer formulation is coated out of a solvent mixture of methyl ethyl ketone (MEK), 1-methoxypropan-2-ol (PGME),  $\gamma$ -butyrolactone (BLO), and water, a mixture of diethyl ketone (DEK), water, 10 methyl lactate, and  $\gamma$ -butyrolactone BLO, or a mixture of methyl lactate, methanol, and dioxolane. The outer layer formulation is generally coated out of DEK, a mixture of DEK and 1-methoxy-2-propyl acetate, a mixture of 1,3-dioxolane, 1-methoxypropan-2-ol (PGME),  $\gamma$ -butyrolactone (BLO), and water, a mixture of MEK and PGME, or a mixture of DEK and acetone.

Alternatively, the inner and outer layers may be applied by conventional extrusion coating methods from melt mixtures of the respective layer compositions. Typically such melt mixtures contain no volatile organic solvents.

Intermediate drying steps may be used between applications of the various layer formulations to remove solvent(s) before coating other formulations. Drying steps may also help in preventing the mixing of the various layers.

Representative methods for preparing imageable elements of this invention are shown in the Examples below.

The imageable elements have any useful form including, but not limited to, printing plate precursors, printing cylinders, printing sleeves and printing tapes (including flexible printing webs). Preferably, the imageable members are printing plate precursors to provide lithographic printing plates.

Printing plate precursors can be of any useful size and shape (for example, square or rectangular) having the requisite inner and outer layers disposed on a suitable substrate. 35 Printing cylinders and sleeves are known as rotary printing members having the substrate and inner and outer layers in a cylindrical form. Hollow or solid metal cores can be used as substrates for printing sleeves.

#### 40 Imaging and Development

During use, the imageable element is exposed to a suitable source of imaging radiation (such as infrared radiation) using a laser at a wavelength of from about 600 to about 1500 nm and preferably from about 600 to about 1200 nm. 45 The lasers used to expose the imaging member of this invention are preferably diode lasers, because of the reliability and low maintenance of diode laser systems, but other lasers such as gas or solid-state lasers may also be used. The combination of power, intensity and exposure time for laser imaging would be readily apparent to one skilled in the art. Presently, high performance lasers or laser diodes used in commercially available imagesetters emit infrared radiation at a wavelength of from about 800 to about 850 nm or from about 1040 to about 1120 nm.

55 The imaging apparatus can function solely as a platesetter or it can be incorporated directly into a lithographic printing press. In the latter case, printing may commence immediately after imaging, thereby reducing press set-up time considerably. The imaging apparatus can be configured as a flatbed recorder or as a drum recorder, with the imageable member mounted to the interior or exterior cylindrical surface of the drum. Examples of useful imaging apparatus is available as models of Creo Trendsetter® imagesetters available from Creo Corporation (a subsidiary of Eastman 60 Kodak Company, Burnaby, British Columbia, Canada) that contain laser diodes that emit near infrared radiation at a wavelength of about 830 nm. Other suitable imaging sources

## 15

include the Gerber Crescent 42T Platesetter that operates at a wavelength of 1064 nm (available from Gerber Scientific, Chicago, Ill.) and the Screen PlateRite 4300 series or 8600 series platesetters (available from Screen, Chicago, Ill.). Additional useful sources of radiation include direct imaging presses that can be used to image an element while it is attached to the printing plate cylinder. An example of a suitable direct imaging printing press includes the Heidelberg SM74-DI press (available from Heidelberg, Dayton, Ohio).

Imaging energies may be in the range of from about 50 to about 1500 mJ/cm<sup>2</sup>, and preferably from about 75 to about 400 mJ/cm<sup>2</sup>. More preferably, the imaging energy is less than 140 mJ/cm<sup>2</sup> and most preferably, less than 120 mJ/cm<sup>2</sup>.

While laser imaging is preferred in the practice of this invention, imaging can be provided by any other means that provides thermal energy in an imagewise fashion. For example, imaging can be accomplished using a thermoresistive head (thermal printing head) in what is known as "thermal printing" as described for example in U.S. Pat. No. 5,488,025 (Martin et al.) and as used in thermal fax machines and sublimation printers. Thermal print heads are commercially available (for example, as Fujitsu Thermal Head FTP-040 MCS001 and TDK Thermal Head F415 HH7-1089).

In any case, direct digital imaging is generally used for imaging. The image signals are stored as a bitmap data file on a computer. The bitmap data files are constructed to define the hue of the color as well as screen frequencies and angles.

Imaging of the imageable element produces an imaged element that comprises a latent image of imaged (exposed) and non-imaged (non-exposed) regions. Developing the imaged element with a suitable alkaline developer removes the exposed regions of the outer layer and the layers (including the inner layer) underneath it, and exposing the hydrophilic surface of the substrate. Thus, the imageable element is "positive-working". The exposed (or imaged) regions of the hydrophilic surface repel ink while the unexposed (or non-imaged) regions of the outer layer accept ink.

More particularly, development is carried out for a time sufficient to remove the imaged (exposed) regions of the outer layer and underlying layers, but not long enough to remove the non-imaged (non-exposed) regions of the outer layer. Thus, the imaged (exposed) regions of the outer layer are described as being "soluble" or "removable" in the alkaline developer because they are removed, dissolved, or dispersed within the alkaline developer more readily than the non-imaged (non-exposed) regions of the outer layer. Thus, the term "soluble" also means "dispersible" or "removable".

The imaged elements are generally developed using conventional processing conditions. Both aqueous alkaline developers and solvent-based developers (that are preferred) can be used.

Aqueous alkaline developers generally have a pH of at least 7 and preferably of at least 11. Useful alkaline aqueous developers include 3000 Developer, 9000 Developer, GoldStar™ Developer, GreenStar Developer, ThermalPro Developer, Protherm® Developer, MX1813 Developer, and MX1710 Developer (all available from Eastman Kodak Company). These compositions also generally include surfactants, chelating agents (such as salts of ethylenediaminetetraacetic acid), and alkaline components (such as inorganic metasilicates, organic metasilicates, hydroxides, and bicarbonates).

## 16

Solvent-based developers are generally single-phase solutions of one or more organic solvents that are miscible with water. Useful organic solvents include the reaction products of phenol with ethylene oxide and propylene oxide [such as 5 ethylene glycol phenyl ether (phenoxyethanol)], benzyl alcohol, esters of ethylene glycol and of propylene glycol with acids having 6 or less carbon atoms, and ethers of ethylene glycol, diethylene glycol, and of propylene glycol with alkyl groups having 6 or less carbon atoms, such as 10 2-ethylethanol and 2-butoxyethanol. The organic solvent(s) is generally present in an amount of from about 0.5 to about 15% based on total developer weight. It is particularly desirable that the alkaline developer contain one or more thiosulfate salts or amino compounds that include an alkyl 15 group that is substituted with a hydrophilic group such as a hydroxy group, polyethylene oxide chain, or an acidic group having a pKa less than 7 (more preferably less than 5) or their corresponding salts (such as carboxy, sulfo, sulfonate, 20 sulfate, phosphonic acid, and phosphate groups). Particularly useful amino compounds of this type include, but are not limited to, monoethanolamine, diethanolamine, glycine, alanine, aminoethylsulfonic acid and its salts, aminopropylsulfonic acid and its salts, and Jeffamine compounds (for 25 example, an amino-terminated polyethylene oxide). The solvent-based developers can have an alkaline, neutral, or slightly acidic pH. Preferably, they are alkaline in pH.

Representative solvent-based alkaline developers include ND-1 Developer, 955 Developer, and 956 Developer (available from Eastman Kodak Company).

Generally, the alkaline developer is applied to the imaged element by rubbing or wiping the outer layer with an applicator containing the developer. Alternatively, the imaged element can be brushed with the developer or the developer may be applied by spraying the outer layer with sufficient force to remove the exposed regions. Still again, the imaged element can be immersed in the developer. In all instances, a developed image is produced in a lithographic printing plate having excellent resistance to press room chemicals.

Following development, the imaged element can be rinsed with water and dried in a suitable fashion. The dried element can also be treated with a conventional gumming solution (preferably gum arabic).

## Post-Development Baking

The imaged and developed element is preferably baked (or cured) in a postbake operation that can be carried out to increase run length of the resulting imaged element. Baking can be carried out in a suitable oven, for example at a temperature of less than 300° C. and preferably at less than 250° C. for from about 2 to about 10 minutes. Most preferably, the baking is done very quickly at a temperature of from about 160 to about 220° C. for from about 2 to about 5 minutes.

Alternatively, the imaged and developed element (for example, printing plate) can be "baked" or cured by overall exposure to IR radiation at a wavelength of from about 800 to about 850 nm. This exposure creates conditions that enable very controllable baking effects with minimal distortion. For example, the imaged and developed element (for example, printing plate) can be passed through a commercial QuickBake 1250 oven (available from Eastman Kodak Company) at 4 feet (1.3 m) per minute at the 45% power setting of an infrared lamp to achieve a similar baking result from heating the element in an oven at 200° C. for 2 minutes.

## Printing

Printing can be carried out by applying a lithographic ink and fountain solution to the printing surface of the imaged element. The ink is taken up by the non-imaged (non-exposed or non-removed) regions of the outer layer and the fountain solution is taken up by the hydrophilic surface of the substrate revealed by the imaging and development process. The ink is then transferred to a suitable receiving material (such as cloth, paper, metal, glass, or plastic) to provide a desired impression of the image thereon. If desired, an intermediate "blanket" roller can be used to transfer the ink from the imaged member to the receiving material. The imaged members can be cleaned between impressions, if desired, using conventional cleaning means and chemicals.

The following examples are provided to illustrate the practice of the invention but are by no means intended to limit the invention in any manner.

## Materials and Methods Used in the Examples:

The materials described below were used in the examples. Unless otherwise indicated, the chemical components can be obtained from a number of commercial sources including Aldrich Chemical Company (Milwaukee, Wis.).

BLO represents  $\gamma$ -butyrolactone.

Byk® 307 is a polyethoxylated dimethyl polysiloxane copolymer that was obtained from Byk Chemie (Wallingford, Conn.) in a 25 wt. % xylene/methoxypropyl acetate solution.

D11 dye is ethanaminium, N-[4-[(4-(diethylamino)phenyl)[4-(ethylamino)-1-naphthalenyl]methylene]-2,5-cyclohexadien-1-ylidene]-N-ethyl-, salt with 5-benzoyl-4-hydroxy-2-methoxybenzenesulfonic acid (1:1) as supplied by PCAS (Longjumeau, France).

DAA represents diacetone alcohol.

DEK represents diethyl ketone.

956 Developer is an organic solvent based (phenoxyethanol) alkaline negative developer that is available from Eastman Kodak Company (Rochester, N.Y.).

DMAC represents N,N-dimethyl acetamide.

Ethyl violet is C.I. 42600 (CAS 2390-59-2,  $\lambda_{max}$ =596 nm) having a formula of  $(p\text{-}(\text{CH}_3\text{CH}_2)_2\text{NC}_6\text{H}_4)_3\text{C}^+\text{Cl}^-$ .

IR Dye A is represented by the following formula:

IR Dye A



MEK represents methyl ethyl ketone.

N-15 represents a p/m-cresol novolak.

P-3000 represents the reaction product of 1,2-naphthoquinone-5-sulfonyl chloride with pyrogallol/acetone condensate (PCAS, Longjumeau, France).

PD-140 is a cresol/formaldehyde novolac resin (75:25 m-cresol/-p-cresol) (Borden Chemical, Louisville, Ky.).

PGME represents 1-methoxypropan-2-ol (or Dowanol PM).

PMI represents N-phenylmaleimide.

RX-04 represents a copolymer derived from styrene and maleic anhydride that was obtained from Gifu (Japan).

Vazo-64 is azobisisobutyronitrile ("AIBN") that was obtained from DuPont (Wilmington, Del.).

Synthesis of N-(4-Carboxyphenyl)methacrylamide (N-BAMAAm):

Acetonitrile (300 ml), methacrylic acid (47.6 g), and ethyl chloroformate (60.05 g) were added in 2-liter 4-neck ground glass flask, equipped with a heating mantle, temperature controller, mechanical glass stirrer, condenser, pressure equalized addition funnel and nitrogen inlet. Triethylamine (55.8 g) was then added slowly at room temperature over one hour while maintaining the reaction temperature maximum at 40° C. The reaction mixture was then stirred for an additional one hour at room temperature. Triethylamine hydrochloride salt was removed and theoretical amount of

TEA:HCl salt was obtained. The mother liquor was placed back into the flask and 4-amino benzoic acid (68.55 g) was added. The reaction mixture was then heated to 50° C. and kept there for 3 hours. The mixture was precipitated in 2.5 liters of 0.1N HCl solution and washed with 1.25 liters of water. The powder was collected by filtration and dried in vacuum oven below 40° C. overnight.

Synthesis of Polymer A:

Dimethylacetamide (65 g), N-BAMAAm (6.5 g), acrylonitrile (8.4 g), methacrylamide (1.7 g), N-phenyl maleimide (0.9 g), and Vazo-64 (0.175 g) were added to a 500 ml 4-neck ground glass flask, equipped with a heating mantle, temperature controller, mechanical stirrer, condenser, pressure equalized addition funnel and nitrogen inlet. The reaction mixture was heated to 80° C. under a nitrogen atmosphere. Then a pre-mixture of dimethylacetamide (100 g), N-BAMAAm (19.4 g), acrylonitrile (25.2 g), methacrylamide (5.3 g), N-phenyl maleimide (2.6 g), and Vazo-64 (0.35 g) were added over two hours at 80° C. The reaction was continued another eight hours and Vazo 64 (0.35 g) was added two more times. The polymer conversion was >99% based on a determination of percent of non-volatiles. The weight ratio of the resulting N-BAMAAm/-AN/methacrylamide/N-phenyl maleimide polymer was 37:48:10:5. The viscosity (G.H'33) was G+ (~170 cps) at 30% non-volatiles in DMAC.

The resin solution was precipitated in powder form using ethanol/water (60:40) using Lab Dispersator (4000 RPM) and filtered, and the slurry was re-dissolved in ethanol and filtered. The resulting powder was dried at room temperature for 48 hours. The resulting yield was 85% and the polymer acid number was 94.4 (actual) versus 95 (theoretical).

Synthesis of Polymer B:

Vazo-64 (0.75 g), PMI (18 g), acrylonitrile (28.8 g), methacrylic acid (MAA, 7.2 g), ethylene glycol methacrylate phosphate (6 g), and DMAc (240 g) were placed in a 500 ml 3-necked flask, equipped with magnetic stirring, condenser, temperature controller and N<sub>2</sub> inlet. The reaction mixture was heated to 60° C. and stirred under N<sub>2</sub> protection for 6 hours, and then Vazo-64 (0.2 g) was added and the reaction was continued overnight. The reaction mixture contained 20% N.V and was slowly dropped into 2000 ml of n-propanol and a precipitate was formed, filtered, and washed with another 400 ml of n-propanol. After filtration and drying at below 50° C., 31 g of solid polymer were obtained.

19

## Synthesis of Polymer C:

Methyl cellosolve (199.8 g), N-methoxymethyl methacrylamide (18 g), benzyl methacrylate (11.4 g), methacrylic acid (3 g), dodecyl mercaptan (0.075 g), and Vazo-64 (0.6 g) were added to 500 ml 4-neck ground glass flask, equipped with a heating mantle, temperature controller, mechanical stirrer, condenser, pressure equalized addition funnel and nitrogen inlet. The reaction mixture was heated to 80° C. under nitrogen atmosphere. Then, a pre-mixture of N-methoxymethyl methacrylamide (55 g), benzyl methacrylate (34 g), methacrylic acid (9 g), dodecyl mercaptan (0.225 g), and Vazo-64 (1.2 g) were added over two hours at 80° C. The reaction was continued another eight hours and Vazo 64 (0.35 g) was added two more times. The polymer conversion was >99% based on determination of percent of non-volatiles. The weight ratio of N-methoxymethyl methacrylamide/benzyl methacrylate/methacrylic acid in the polymer was 56/34/8.9/2. The resin solution was precipitated in powder form using DI water/Ice (3:1) and a Lab Dispersor (4000 RPM) and then filtered. The resulting powder was dried at room temperature for 24 hours. The next day, a tray containing the polymer was placed in oven at 110° F. (43° C.) for two additional days. The yield was 95% and polymer acid number was 58 (actual) versus 58.8 (theoretical).

## Synthesis of Polymer E:

Arcosolve PM Acetate (propylene glycol methyl ether acetate from Arco Chemicals, 116 g), m-TMI (33.80 g 1-(1-isocyanate-1 methyl)ethyl-3-(1-methyl), ethenyl benzene, from Cytec Industries), ethyl acrylate (3.80 g), and t-butyl peroxy benzoate (6 g) were added to a 500 ml 4-neck ground glass flask, equipped with a heating mantle, temperature controller, mechanical stirrer, condenser, pressure equalized addition funnel and nitrogen inlet. The reaction mixture was heated to 120° C. under nitrogen atmosphere. Then, a pre-mixture of m-TMI (101.20 g), ethyl acrylate (11.20 g), and of t-butyl peroxy benzoate (12 g, Aldrich Chemicals) was added over 2-hours at 120° C. After the addition was complete, an additional 9 g of t-butyl peroxy benzoate were added in two portions. The reaction was completed to theoretical percent non-volatiles (60%) in 16 hours. Then, a partial batch of this solution (118 g) containing free —NCO group was further reacted with p-amino phenol (26.65 g) at 1:1.02 equivalent ratio. The reaction was monitored by IR-spectroscopy for disappearance of —NCO group at 2275 cm<sup>-1</sup> and was completed by heating to 40° C. The resulting product was a copolymer of ethyl acrylate and the urea adduct of m-TMI/p-amino phenol and was precipitated in powder form using water/ice, filtered, and dried at room temperature.

## Synthesis of Polymer F:

Dimethylacetamide (61.0 g), 4-hydroxy phenyl methacrylamide (2.5 g), acrylonitrile (6.0 g), methacrylamide (1.25 g), n-phenyl maleimide (2.75 g), and Vazo-64 (0.125 g) were added to a 250 ml 4-neck ground glass flask, equipped with a heating mantle, temperature controller, mechanical stirrer, condenser, pressure equalized addition funnel and nitrogen inlet. The reaction mixture was heated to 80° C. under nitrogen atmosphere. Then, pre-mixture of 70.0 g of dimethylacetamide (70.0 g), hydroxy phenyl methacrylamide (7.5 g), acrylonitrile (18.0 g), methacrylamide (3.75 g), n-phenyl maleimide (8.25 g), and Vazo-64 (0.25 g) were added over two hours at 80° C. Reaction was continued another sixteen hours during which time Vazo-64 was added two more times (total amount=0.38 g). The polymer conversion was >98% based on determination of percent of non-volatiles. The viscosity (G.H'33) was A (~50 cps). The

20

resin solution was precipitated in powder form using 5000 g of Ice/water (1:3) using a Lab Dispersor (4000 RPM). The powder was dried at room temperature for 48 hours and two days at 43° C. to provide a yield of 95%.

## 5 Synthesis of Polymer G:

Dimethylacetamide (65 g), acrylonitrile (8.4 g), methacrylamide (3.1 g), n-phenyl maleimide (3.1 g), methacrylic acid (2.9 g), and Vazo-64 (0.175 g) were added to a 500 ml 4-neck ground glass flask, equipped with a heating mantle, temperature controller, mechanical stirrer, condenser, pressure equalized addition funnel, and nitrogen inlet. The reaction mixture was heated to 80° C. under nitrogen atmosphere. Then, a pre-mixture of dimethylacetamide (100 g), acrylonitrile (25.2 g), methacrylamide (9.3 g), n-phenyl maleimide (9.3 g), methacrylic acid (8.7 g), and Vazo-64 (0.525 g) were added over two hours at 80° C. The reaction was continued another fourteen hours during which time Vazo-64 was added two more times (total amount=0.5 g). The polymer conversion was >98% based on determination of percent of non-volatiles. The viscosity (G.H'33) was F (140 cps). The polymer solution (30% non-volatile in dimethylacetamide) was directly used in the inner layer formulation.

## 10 15 20 25 30 35 40 45 50 55 60 65 Synthesis of Polymer H:

Dimethylacetamide (100.0 g), acrylonitrile (12.0 g), methacrylamide (5.5 g), n-phenyl maleimide (5.5 g), methacrylic acid (1.25 g), and Vazo-64 (0.25 g) were added to a 500 ml 4-neck ground glass flask, equipped with a heating mantle, temperature controller, mechanical stirrer, condenser, pressure equalized addition funnel, and nitrogen inlet. The reaction mixture was heated to 80° C. under a nitrogen atmosphere. Then, a pre-mixture of dimethylacetamide (136.66 g), acrylonitrile (36.0 g), methacrylamide (18.0 g), n-phenyl maleimide (18.0 g), methacrylic acid (3.75 g), and Vazo-64 (0.5 g) were added over two hours at 80° C. Reaction was continued another fourteen hours during which time Vazo 64 was added two more times (total amount=0.6 g). The polymer conversion was >97% based on determination of percent of non-volatiles. The viscosity (G.H'33) was D (100 cps). The polymer solution (30% non-volatile in dimethylacetamide) was directly used in the inner layer formulation.

## Synthesis of Polymer I:

Dimethylacetamide (100.0 g), N-BAMAAm (9.25 g), methacrylamide (3.6 g), n-phenyl maleimide (7.2 g), styrene (5.0 g), and Vazo-64 (0.25 g) were added to a 500 ml 4-neck ground glass flask, equipped with a heating mantle, temperature controller, mechanical stirrer, condenser, pressure equalized addition funnel, and nitrogen inlet. The reaction mixture was heated to 80° C. under a nitrogen atmosphere. Then a pre-mixture of dimethylacetamide (136.66 g), N-BAMAAm (27.75 g), methacrylamide (10.7 g), n-phenyl maleimide (21.5 g), styrene (15.0 g), and Vazo-64 (0.5 g) were added over two hours at 80° C. Reaction was continued another six hours during which time Vazo-64 was added two more times (total amount=0.25 g). The polymer conversion was >98% based on determination of percent of non-volatiles. The viscosity (G.H'33) was J (~240 cps). The polymer solution (30% non-volatile in dimethylacetamide) was directly used in the inner layer formulation.

## Synthesis of Polymer J:

Vazo-64 (0.4 g), n-phenyl maleimide (14 g), methacrylic acid (3 g), ethylene glycol methacrylate phosphate (3 g), and N,N-dimethylacetamide (60 g) were placed in a 250-ml 3-necked flask, equipped with magnetic stirring, condenser,

21

temperature controller, and  $N_2$  inlet. The reaction mixture was heated to 80° C. and stirred under  $N_2$  protection overnight (16 h). The polymer conversion was >90% based on determination of percent of non-volatiles. The reaction mixture was then slowly dropped into 3000 ml of water while stirring. The resulting precipitate was filtered and washed with 200 ml of propanol and filtered and dried at 50° C. for 3 hours to provide 16 g of solid powder.

## EXAMPLE 1

An imageable element of the present invention was prepared as follows:

An inner layer coating formulation was prepared by dissolving 3.834 g of Polymer A and 2.13 g of Polymer C in a solvent mixture of 9.27 g of BLO, 13.9 g of PGME, 60.27 g of MEK, and 9.27 g of water. IR Dye A (1.06 g) was then added to this solution followed by addition of 0.211 g of Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of PD-140, 0.014 g of ethyl violet, 0.149 g of 10% Byk® 307 in 85.38 g of DEK, and 9.48 g of acetone. This formulation was coated over the inner layer formulation described above to provide a dry outer layer weight of 0.5 g/m<sup>2</sup>.

The dried imageable element was thermally imaged on a commercially available Creo Trendsetter 3244 (Creo, a subsidiary of Eastman Kodak Company, Burnaby, BC, Canada) having a laser diode array emitting at 830 nm with a variety of exposure energies from 60 to 140 mJ/cm<sup>2</sup>. The resulting imaged element was developed with 956 Developer in a commercial processor. The minimum energy to achieve a desired image was about 100 mJ/cm<sup>2</sup>.

The following two Bakeability (curability) tests were used to evaluate the imaged and developed printing plates, and particularly to evaluate the curability of the inner layer compositions:

(1) Heating the element in a convection oven at 190° C. for 2 minutes,

(2) Passing the element through a commercial QuickBake 1250 oven (available from Eastman Kodak Company) at 4 feet/minute (1.2 m/min.), with 30% power setting of an infrared lamp.

A PS plate image remover, PE-3S (from Dainippon Ink Co., Japan), was then applied onto the above baked (cured) coat surfaces at regular intervals up to 10 minutes at ambient temperature. For both baking methods, no obvious coating damage was seen on the areas that were treated with PE-3S up to 5 minutes.

## COMPARATIVE EXAMPLE 1

An imageable element outside of the present invention was prepared as follows:

An inner layer coating formulation was prepared by dissolving 6.01 g of Polymer A in a solvent mixture of 9.27 g of BLO, 13.9 g of PGME, 60.27 g of MEK, and 9.27 g of water. IR Dye A (1.06 g) was then added to this solution followed by addition of 0.211 g of Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of Polymer E, 0.014 g of ethyl violet, 0.149 g of 10% Byk® 307 in 85.38 g of DEK and 9.48 g of acetone.

22

This formulation was coated over the inner layer formulation described above to provide a dry outer layer weight of 0.5 g/m<sup>2</sup>.

The dried imageable element was thermally imaged and processed as described in Example 1. The minimum energy to achieve a desired image was >180 mJ/cm<sup>2</sup>.

The two Bakeability tests described above for Example 1 were carried out. For both baking methods, severe coating damage was seen on the areas that were treated with PE-3S from 1 to 5 minutes. Another test was carried out by heating the imaged element in an oven at 230° C. for 8 minutes. The resulting baked element was not damaged by the PE-3S for up to 5 minutes.

## EXAMPLE 2

An imageable element of the present invention was prepared as follows:

An inner layer coating formulation was prepared by dissolving 3.834 g of Polymer B and 2.13 g of Polymer C in a solvent mixture of 9.27 g of BLO, 13.9 g of PGME, 60.26 g of MEK, and 9.27 g of water. IR Dye A (1.06 g) was then added to this solution followed by addition of 0.211 g of Byk® 307 and 0.0497 g of D-11 dye. The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of Polymer E, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The dried imageable element was thermally imaged and processed as described in Example 1. The minimum energy to achieve a desired image was about 100 mJ/cm<sup>2</sup>.

The two Bakeability tests described in Example 1 were carried out. For both baking methods, no obvious coating damage was seen on the areas that were treated with PE-3S up to 5 minutes.

## COMPARATIVE EXAMPLE 2

An imageable element outside of the present invention was prepared as follows:

An inner layer coating formulation was prepared by dissolving 6.014 g of Polymer B in a solvent mixture of 9.27 g of BLO, 13.9 g of PGME, 60.26 g of MEK, and 9.27 g of water. IR Dye A (1.06 g) was then added to this solution followed by addition of 0.211 g of Byk® 307. The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of Polymer E, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The dried imageable element was thermally imaged and processed as described in Example 1. The minimum energy to achieve a desired image was >180 mJ/cm<sup>2</sup>.

The two Bakeability tests described in Example 1 were also carried out. For both baking methods, severe coating damage was seen on the areas that were treated with PE-3S for 1 to 5 minutes. Another test was carried out by heating

23

the imaged element in an oven at 230° C. for 8 minutes. The resulting baked element was not damaged by the PE-3S for up to 5 minutes.

## EXAMPLE 3

An imageable element of the present invention was prepared as follows:

An inner layer coating formulation was prepared by dissolving 3.834 g of Polymer B and 2.13 g of Polymer C in a solvent mixture of 9.27 g of BLO, 13.9 g of PGME, 60.26 g of MEK, and 9.27 g of water. IR Dye A (1.06 g) was then added to this solution followed by addition of 0.211 g of Byk® 307 and 0.0497 g of D-11 dye. The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of N-15, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The dried imageable element was thermally imaged and processed as described in Example 1. The minimum energy to achieve a desired image was about 100 mJ/cm<sup>2</sup>.

The two Bakeability tests described in Example 1 were carried out. For both baking methods, no obvious coating damage was seen on the areas that were treated with PE-3S up to 5 minutes.

## EXAMPLE 4

Another imageable element of the present invention was prepared as follows:

An inner layer coating formulation was prepared by dissolving 3.834 g of Polymer B and 2.13 g of Polymer C in a solvent mixture of 9.27 g of BLO, 13.9 g of Dowanol PM, 60.26 g of MEK, and 9.27 g of water. IR Dye A (1.06 g) was then added to this solution followed by addition of 0.211 g of Byk® 307 and 0.0497 g of D-11 dye. The resulting solution was coated onto a grained and anodized aluminum lithographic substrate to provide a 1.5 g/m<sup>2</sup> dry inner layer weight.

An outer layer formulation was prepared by mixing 4.971 g of RX-04, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The dried imageable element was thermally imaged and processed as described in Example 1. The minimum energy to achieve a desired image was about 100 mJ/cm<sup>2</sup>.

The two Bakeability tests described in Example 1 were carried out. For both baking methods, no obvious coating damage was seen on the areas that were treated with PE-3S up to 5 minutes.

## COMPARATIVE EXAMPLE 3

Another imageable element outside of the present invention was prepared as follows:

An inner layer coating formulation was prepared by dissolving 3.834 g of Polymer F and 2.13 g of Polymer C in a solvent mixture of 9.27 g of BLO, 13.9 g of PGME, 60.27 g of MEK, and 9.27 g of water. IR Dye A (1.06 g) was then added to this solution followed by addition of 0.211 g of

24

Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of PD-140, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The dried imageable element was thermally imaged and processed as described in Example 1. However, the imaged element was not processable in 956 Developer.

The Bakeability tests described above in Example 1 were carried out. When the element was heated in a convection oven at 190° C. for 2 minutes, severe coating damage was seen on the areas that were treated with PE-3S for 1 to 5 minutes. The test was repeated by heating the imaged element at 220° C. for 2 minutes, and the resulting baked element was also damaged by contact with the PE-3S for 1 to 5 minutes.

## EXAMPLE 5

An imageable element of the present invention was prepared as follows:

An inner layer coating formulation was prepared by dissolving 12.8 g of Polymer G (30% in DMAC) and 2.13 g of Polymer C in a solvent mixture of 9.27 g of BLO, 13.9 g of PGME, 60.27 g of MEK, and 9.27 g of water. IR Dye A (1.06 g) was then added to this solution followed by addition of 0.211 g of Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of PD-140, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The dried imageable element was thermally imaged and processed as described in Example 1. The minimum energy to achieve a desired image was about 150 mJ/cm<sup>2</sup>.

The two Bakeability tests described in Example 1 were carried out. For both tests, no obvious coating damage was seen on the areas that were treated with PE-3S for up to 5 minutes.

## EXAMPLE 6

An imageable element of the present invention was prepared as follows:

An inner layer coating formulation was prepared by dissolving 12.8 g of Polymer H (30% in DMAC) and 2.13 g of Polymer C in a solvent mixture of 9.27 g of BLO, 13.9 g of PGME, 60.27 g of MEK, and 9.27 g of water. IR Dye A (1.06 g) was then added to this solution followed by addition of 0.211 g of Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of PD-140, 0.014 g of ethyl violet, 0.149 g of 10% Byk® 307 in 85.38 g of DEK and 9.48 g of

## 25

acetone. This formulation was coated over the inner layer formulation described above to provide a dry outer layer weight of 0.5 g/m<sup>2</sup>.

The two Bakeability tests described in Example 1 were carried out. For both tests, only slight coating damage was seen on the areas that were treated with PE-3S for 4 to 5 minutes.

## EXAMPLE 7

Another imageable element of the present invention was prepared as follows:

An inner layer coating formulation was prepared by dissolving 12.8 g of Polymer I (30% in DMAc) and 2.13 g of Polymer C in a solvent mixture of 9.27 g of BLO, 13.9 g of PGME, 60.27 g of MEK, and 9.27 g of water. IR Dye A (1.06 g) was then added to this solution followed by addition of 0.211 g of Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of PD-140, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The two Bakeability tests described in Example 1 were carried out. For both tests, only slight coating damage was seen on the areas that were treated with PE-3S for 3 to 4 minutes.

## EXAMPLE 8

Still another imageable element of the present invention was prepared as follows:

An inner layer coating formulation was prepared by dissolving 3.84 g of Polymer J and 2.13 g of Polymer C in a solvent mixture of 9.27 g of BLO, 13.9 g of PGME, 60.27 g of MEK, and 9.27 g of water. IR Dye A (1.06 g) was then added to this solution followed by addition of 0.211 g of Byk® 307 (10% solution in PGME). The resulting solution was coated onto a grained and anodized aluminum lithographic substrate to provide a 1.5 g/m<sup>2</sup> dry inner layer weight.

An outer layer formulation was prepared by mixing 1.503 g of P-3000, 3.469 g of PD-140, 0.014 g of ethyl violet, 0.149 g of 10% Byk® 307 in 85.38 g of DEK and 9.48 g of acetone. This formulation was coated over the inner layer formulation described above to provide a dry outer layer weight of 0.5 g/m<sup>2</sup>.

The two Bakeability tests described in Example 1 were carried out. For both tests, only slight coating damage was seen on the areas that were treated with PE-3S for 3 to 4 minutes.

The invention has been described in detail with particular reference to certain preferred embodiments thereof, but it will be understood that variations and modifications can be effected within the spirit and scope of the invention.

The invention claimed is:

1. A positive-working imageable element comprising a radiation absorbing compound and a substrate having a hydrophilic surface, and having on said substrate, in order: an inner layer composition comprising first and second polymeric binders, and an ink receptive outer layer,

## 26

provided that upon thermal imaging, the exposed regions of said element are removable by an alkaline developer, wherein said first polymeric binder has an acid number of at least 30 and comprises recurring units comprising acidic groups and recurring units derived from a (meth) acrylonitrile, and

said second polymeric binder comprises recurring units derived from an N-alkoxymethyl (alkyl)acrylamide, alkoxyethyl (alkyl)acrylate, or hydroxymethyl (alkyl) acrylamide.

2. The element of claim 1 wherein said inner layer composition is curable upon heating at from about 160 to about 220° C. for from about 2 to about 5 minutes, or by overall infrared radiation exposure at from about 800 to about 850 nm.

3. The element of claim 1 wherein said first polymeric binder has an acid number of at least 50.

4. The element of claim 1 wherein said first polymeric binder comprises recurring units derived from a (meth) acrylic acid, carboxyphenyl (meth)acrylamide, an alkylene glycol (meth)acrylate phosphate, or a combination thereof.

5. The element of claim 1 wherein said second polymeric binder comprises recurring units derived from a methoxymethyl (meth)acrylamide, hydroxymethyl (meth)acrylamide, methoxymethyl (meth)acrylate, or any combination thereof.

6. The element of claim 1 wherein said first polymeric binder comprises recurring units derived from a 4-carboxyphenyl (meth)acrylamide, an ethylene glycol (meth)acrylate phosphate, (meth)acrylic acid, or a combination thereof, and said second polymeric binder comprises recurring units derived from an N-alkoxymethyl (meth)acrylamide.

7. The imageable element of claim 1 wherein the weight ratio of said first polymeric binder to said second polymeric binder in said inner layer is from about 0.2:1 to about 20:1.

8. The imageable element of claim 1 wherein said first polymeric binder is represented by the following Structure (I):



wherein A represents recurring units derived from a (meth) acrylic acid, carboxyphenyl (alkyl)acrylamide, an (alkyl)acrylate phosphate, or a combination thereof, B represents recurring units derived from one or more different ethylenically unsaturated polymerizable monomers other than those used to obtain the A recurring units and including recurring units derived from (meth)acrylonitrile, x is from about 1 to about 70 mol %, and y is from about 30 to about 99 mol %.

9. The imageable element of claim 8 wherein x is from about 5 to about 50 mol %, and y is from about 50 to about 95 mol %, based on total recurring units.

10. The imageable element of claim 8 wherein B is derived from one or more (meth)acrylonitriles, and optionally one or more (meth)acrylic acid esters, (meth)acrylamides, vinyl carbazole, styrene and styrenic derivatives thereof, N-substituted maleimides, maleic anhydride, vinyl acetate, vinyl ketones, vinyl pyridine, N-vinyl pyrrolidones, 1-vinylimidazole, vinyl polyalkylsilanes, or combinations thereof.

11. The imageable element of claim 1 wherein said second polymeric binder is represented by the following Structure (II):



wherein C represents recurring units derived from an N-alkoxymethyl (alkyl)acrylamide, alkoxyethyl (alkyl)acrylate, hydroxymethyl (alkyl)acrylamide, or any combination thereof, D represents recurring units derived from one

or more different ethylenically unsaturated polymerizable monomers other than those used to obtain the C recurring units, w is from about 5 to about 80 mol %, and z is from about 20 to about 95 mol %, based on total recurring units.

12. The imageable element of claim 11 wherein w is from about 10 to about 60 mol %, z is from about 40 to about 90 mol %, based on total recurring units, and D is derived from one or more (meth)acrylic acid esters, (meth)acrylonitriles, (meth)acrylamides, vinyl carbazole, styrene and styrenic derivatives thereof, N-substituted maleimides, maleic anhydride, vinyl acetate, vinyl ketones, vinyl pyridine, N-vinyl pyrrolidones, 1-vinylimidazole, vinyl monomers having carboxy groups, vinyl polyalkylsilanes, or combinations thereof.

13. The imageable element of claim 1 wherein the total amount of said first and second polymeric binders is from about 50 to about 99%, said first polymeric binder is present in an amount of from about 20 to about 90 weight % and said second polymeric binder is present in an amount of from about 5 to about 80 weight %, all based on the total dry weight of said inner layer.

14. The imageable element of claim 1 wherein said radiation absorbing compound is an infrared absorbing compound that is present in an amount of from about 5 to about 40 weight % based on the total dry weight of said inner layer, and the weight ratio of said first polymeric binder to said second polymeric binder in said inner layer is from about 1:1 to about 10:1.

15. A method for forming an image comprising:

A) thermally imagewise exposing the positive-working imageable element of claim 1, thereby forming an imaged element with exposed and non-exposed regions,

B) contacting said imaged element with an alkaline developer to remove only said exposed regions, and

C) optionally, baking said imaged and developed element.

16. The method of claim 15 wherein said imagewise exposing is carried out using an infrared laser providing radiation at a wavelength of from about 600 to about 1200 nm.

17. The method of claim 15 wherein said imaged and developed element is baked at less than 300° C. for less than 10 minutes.

18. The method of claim 17 wherein said imaged and developed element is baked at from about 160 to about 220° C. for from about 2 to about 5 minutes, or by overall infrared radiation exposure at from about 800 to about 850 nm.

19. The method of claim 15 wherein the total amount of said first and second polymeric binders is from about 50 to about 99% based on total dry inner layer weight, the weight ratio of said first polymeric binder to said second polymeric binder in said inner layer is from about 1:1 to about 10:1, said first polymeric binder is present in an amount of from about 20 to about 80 weight %, and said second polymeric

binder is present in an amount of from about 10 to about 80 weight %, both based on the total dry weight of said inner layer,

said first polymeric binder has an acid number of at least 50 and is represented by the following Structure (I):



wherein A represents recurring units derived from a (meth)acrylic acid, 4-carboxyphenyl methacrylamide, an ethylene glycol methacrylate phosphate, or a combination thereof, B represents recurring units derived from one or more different ethylenically unsaturated polymerizable monomers other than those used to obtain the A recurring units and including recurring units derived from (meth)acrylonitrile, x is from about 5 to about 50 mol %, and y is from about 50 to about 95 mol %,

said second polymeric binder is represented by the following Structure (II):



wherein C represents recurring units derived from an N-alkoxymethyl methacrylamide, w is from about 10 to about 60 mol %, and z is from about 40 to about 90 mol %, based on total recurring units, and D independently represents recurring units derived from one or more of an N-substituted maleimide, N-substituted (meth)acrylamide, unsubstituted (meth)acrylamide, methyl (meth)acrylate, benzyl (meth)acrylate, (meth)acrylonitrile, (meth)acrylic acid, a styrenic monomer, or combinations thereof, and

said radiation absorbing compound is present exclusively in said inner layer in an amount of from about 7 to about 20 weight %, and is an IR dye having a  $\lambda_{max}$  of from about 700 to about 1200 nm.

20. An imaged element obtained from the method of claim 15.

21. A positive-working imageable element comprising a radiation absorbing compound and a substrate having a hydrophilic surface, and having on said substrate, in order: an inner layer composition comprising first and second polymeric binders, and an ink receptive outer layer,

provided that upon thermal imaging, the exposed regions of said element are removable by an alkaline developer, wherein said first polymeric binder has an acid number of at least 30 and comprises recurring units comprising acidic groups which recurring units are derived from carboxyphenyl (meth)acrylamide, an alkylene glycol (meth)acrylate phosphate, or a combination thereof, and

said second polymeric binder comprises recurring units derived from an N-alkoxymethyl (alkyl)acrylamide, alkoxymethyl (alkyl)acrylate, or hydroxymethyl (alkyl)acrylamide.

\* \* \* \* \*